

# UNITED STATES PATENT OFFICE.

CARL AUER VON WELSBACH, OF VIENNA, AUSTRIA-HUNGARY.

## MANUFACTURE OF ELECTRIC FILAMENTS.

1,109,887.

Specification of Letters Patent.

Patented Sept. 8, 1914.

No Drawing.

Application filed August 24, 1899. Serial No. 728,357.

To all whom it may concern:

Be it known that I, DR. CARL AUER VON WELSBACH, a subject of the Emperor of Austria-Hungary, residing at Vienna, Austria-Hungary, have invented or discovered a certain new and useful Improvement in the Manufacture of Electric Filaments, of which the following is a specification.

In a companion application, filed of even date herewith, No. 728,356 I have described certain methods for eliminating from filaments of osmium or osmium alloy, either alone or coated, or otherwise associated with metallic oxids, the occluded gases absorbed by the osmium during a certain stage of its formation. The present application relates to the filaments themselves produced by the practice of the methods referred to, or in any other manner. I find that lamps made of filaments from which those gases have been eliminated, which will not remain occluded in the osmium when the filament is brought to white incandescence, have a substantially perfect and practically lasting vacuum throughout the life of the lamp. In my said companion application I have described various methods for producing filaments having these characteristics. Thus, to produce a filament of pure osmium devoid of said gases, I proceed as follows: When the filament for the bulb is to be of pure osmium, I mount it therein by fusing the bulb to the portion of the lamp which carries the filament and leading-in wires, taking care to first carefully clean the bulb itself. I then fill the bulb with a dry gas, such as nitrogen which will not attack the osmium, while hot, and then, while highly heating the bulb, I exhaust the gases therefrom. Thereupon, I pass a current of dry reducing gases (as, for instance, dry carbonaceous gases) through the bulb and again exhaust, repeating this latter alternate gas-rinsing and exhausting operation several times. Finally, when, after the last gas-rinsing, the subsequent exhausting operation has considerably lowered the pressure in the bulb, I pass an electric current of say 2 or 4 watts per candle, through the filament, sufficient to bring it to a corresponding luminosity, and I then complete the vacuum. The filament thereupon begins to slowly give off its occluded gases, and its luminosity increases until it attains a dazzling whiteness. As soon as it completely ceases to give off

gases, I seal the bulb, whereupon it will be found that the exterior appearance of the filament has not been affected in any particularly noticeable manner, and a substantially perfect vacuum obtained, which will be practically maintained throughout the life of the lamp. If the lamp is to be used in an inclined position, or under circumstances subjecting it to jolts or jars, the filament may be attached to the bulb at any place therein in manner similar to the way in which carbon filaments for high tension lamps are attached.

To eliminate the occluded gases (without materially reducing the oxid) from filaments consisting of a mixture of oxid and osmium and also those wherein the osmium is coated with oxid, I proceed as follows: I first mount the filaments in the bulb, as before, by fusion. I then rinse the bulb by passing a current of dry gas (such as nitrogen) through it and thereupon partially exhaust it. I then pass a current of electricity through the filament sufficient to first raise the filament to a red heat, gradually increasing the current until the filament is raised to a yellowish white heat, in the meantime continuously, or from time to time, increasing the vacuum. During this operation, the filament gives off its occluded gases and a faint glimmering takes place within the bulb for a considerable period. As soon as the development of gas ceases permanently, but not until then, I increase the strength of the current sufficiently to bring the filament to a bright white heat, and, as soon as the resistance becomes constant, I seal the bulb. Care must be taken, in this process, to prevent energetic glimmering, as otherwise the interior of the bulb will be covered with a brownish coating.

The process just described for obtaining said filaments of associated osmium and oxid filaments free from occluded gases may be replaced by the following process which requires less time: An osmium filament is first fastened in the lamp-base with osmium cement, or preferably iridium-osmium cement, as contemplated in my application No. 688,204, filed August 9, 1898, and issued as Patent No. 976,528, Nov. 29, 1910. It is then inserted within a closed receptacle and a vacuum is produced within the receptacle. The filament is then raised to a yellowish white heat by the electric current. As soon

60

65

80

85

90

95

100

105

110

as glimmering begins, nitrogen with some oxidizing agent, as, for instance, small quantities of air, (or, preferably, steam or carbonic acid gas,) or similar gases or vapors, are admitted, for the purpose of uniting with the occluded gases as they are given off by the filament. As soon as this union has taken place, the vessel is filled with dry nitrogen. The filament is then coated with oxids and dried quickly, and the lamp base is united with the bulb, whereupon, to finish the lamp, it is merely necessary to exhaust and seal the bulb.

It will be noted that in the production of a filament of associated osmium and oxid substantially free from occluded gases, the process has been conducted under conditions unfavorable to the reduction of the oxid, in whole or in part by the said gases. That is, the strength of the electric current employed for heating the filament has been such as to expel the occluded gases from the osmium but not sufficient to produce a temperature at which the gases would combine with and reduce the oxid. Thus, according to the first method above described for treating filaments of associated osmium and oxid, the filament is first raised to a red heat and finally to a yellowish white heat, and the occluded gases given off are continuously exhausted by the vacuum pump; and it is not until the development of gas has entirely ceased that a higher temperature is employed. So also in the second method described for producing filaments of associated osmium and oxid devoid of occluded gases, the occluded gases as for instance, hydrogen, carbonic acid, carbon dioxid, and hydrocarbon gases are first eliminated from the osmium filament with which the method is started, before the oxids are applied to said filament. The resulting filament in both cases is, therefore, a filament consisting substantially of osmium either admixed with or coated with an oxid practically unreduced. I may so conduct the operation, however, as to produce a filament wherein the osmium is associated with or coated with a combination of varying composition, varying according to the quantity of oxygen withdrawn from the oxid of the original filament of associated osmium and oxid treated. These combinations are produced either by a partial reduction of the oxid with which the osmium is associated or coated or by a partial oxidation of a metal-osmium filament. Externally these filaments exhibit a nearly metallic appearance and appear to be entirely homogeneous. Their conductivity is, in general greater than that of the filaments of associated osmium and oxid from which they may be produced, but less than that of the metallic osmium alloys. They occlude gases in about the same degree as do the osmium filaments themselves. Heated

to a dazzling white heat *in vacuo* they do not glimmer and resist high temperatures. The production of these last mentioned filaments by the utilization of the occluded gases contained within the osmium has the advantage that not only are said gases quickly and effectually withdrawn from the filament and from the bulb itself by the action of the vacuum pump, whereby the vacuum in the bulb is attained with corresponding rapidity and with the assurance that it will be permanent, but also that the degree of the reduction may be predetermined and controlled with great accuracy. The process of producing the said filaments by obtaining a partial reduction of the oxids by the occluded gases is quite similar to that for the production of the filaments of associated osmium and oxid from which they may be derived. Ordinary filaments of associated osmium and oxid (for instance filaments consisting of osmium associated with thorium oxid) are first mounted, by fusion, in the lamp bulb. The bulb is then rinsed with dry gases and filled therewith, whereupon it is connected with the vacuum pump and the exhausting operation is begun. The filament is then brought to a bright incandescence, the rather high resistance of the filament remaining constant. The development of gas begins and eventually the lamp begins to glimmer. When, after a considerable interval, the development of gas slackens and an almost complete vacuum exists in the bulb, the strength of the current is increased until the filament is brought to a dazzling white heat. Presently the resistance of the filament suddenly sinks, the temperature required for reduction having been reached, whereupon a corresponding resistance must be switched in or the tension of the current must be diminished. The development of gas then ceases and the glimmer becomes extinguished. The resistance gradually sinks still lower, and after some time becomes constant. The filament contracts and the vacuum being completed, the lamp is then to be sealed. According to the quantity of the gases present in the osmium filament at the time of the beginning of the reaction, and according to the quantity of oxid present in the filament itself, the resulting conductibility of the filament is higher or lower. Inasmuch as in practice, it is often desirable to have a high resistance, I preferably give to the filament as high a percentage of oxid as possible. But, in view of the fact that filaments with a high percentage of oxid require for their production high tension currents and inasmuch as this percentage in many cases (particularly for thorium oxid) should not materially exceed fifty per cent, because the conductibility of the original oxid and osmium filaments in the cold diminishes as the percentage of oxid

increases, and with even greater rapidity it is therefore advisable not to give a filament too high an original percentage of oxids, but to afterward saturate it with the oxid 5 and to coat it.

It will be, of course, understood that osmium may be commingled with the oxid in the saturating or coating solution or emulsion. When this process is correctly carried out it has the advantage of making the filaments denser, so that they will not glimmer materially during the subsequent formation period in the lamp. The oxid or mixture of osmium and oxid applied to the 15 filament for the purpose of saturating and coating the same is preferably, in the finest subdivision, made into an emulsion: The filament is thereupon dipped into the emulsion throughout the entire length of the 20 filament excepting the terminal ends thereof to which the leading in wires are to be attached. The filament is then dried and again dipped in the emulsion, again dried &c., until the desired quantity of oxid or 25 osmium and oxid has been added to it. If the quantity to be applied to the filament is rather large, it is advisable at intervals to insert the filament within a protecting gas mixture and to bring it to a white heat 30 therein. In this manner we obtain a core of better conducting oxid and osmium and a coating of less conductivity. Instead of using oxid and osmium filaments, it will, of course, be understood that filaments of pure 35 osmium may be used; in the latter case, however, it is advisable not to make the filaments too dense which may be readily guarded against by making the filament out of lime and osmium paste and by not heating 40 the filament too high subsequently when it is being consolidated. In this instance, the saturation and coating of the filament takes place in the manner just described, and the further treatment of the saturated 45 and coated filament, up to the completion of the lamp, is likewise the same.

I have found that thorium oxid is the oxid best adapted for the production of these filaments of partly reduced oxid and osmium 50 or partly oxidized osmium. It may, however, be entirely or partially replaced by oxid of zirconium, the ytterite earths and similar refractory oxids whose partly reduced oxid when associated with osmium 55 resists the high temperatures employed in practice and these substitute materials may be employed either alone or in admixture with each other in place of the thorium oxid, although, as I have intimated, with less advantage. When oxids of the highest capacity to resist high temperatures are employed, the filament may likewise contain oxids which of themselves would melt or 60 volatilize at white incandescence, as for instance, lime: the greater the percentage of

the oxid which fully resists volatilization, the more firmly will be held the oxid which resists this volatilization to a lesser degree. The admixture of these inferior oxids with the thorium oxid is of advantage when they 70 favorably influence, at white incandescence, the candle power of the filament.

In all of these filaments, osmium may be replaced in part by other platinum metals, as ruthenium, iridium or rhodium, without 75 essentially altering the operation. Such filaments, however, in case they contain considerable quantities of the metals referred to, have not a very high capacity for resisting disintegration. Nevertheless, they are 80 characterized by the remarkable property that, in spite of a considerable percentage in osmium they do not, after a time give off osmium vapors when brought to white incandescence in the open air.

Filaments produced in accordance with the processes hereinbefore set forth are, by reason of the practical elimination of the 85 occluded gases, homogeneous and wholly or substantially free from glimmering when 90 brought to white incandescence.

Having thus described my invention, what I claim is:

1. A filament for electric vacuum lamps, containing osmium, and oxid of a rare metal earth, and a supplemental oxid, said filament containing, at ordinary temperatures, substantially only such gases as remain occluded therein at white incandescence.

2. A filament for electric vacuum lamps, containing osmium, and partly reduced oxid compounds of a supplemental metal.

3. A filament for electric vacuum lamps, containing osmium, and partly reduced oxid 105 compounds of a rare metal earth.

4. A filament for electric vacuum lamps, containing osmium, partly reduced oxid compounds of a rare metal earth, and an oxid of a supplemental metal.

5. A filament for electric vacuum lamps, containing osmium, and partly reduced oxid 110 compounds of thorium.

6. A filament for electric vacuum lamps, containing osmium, and partly reduced oxid 115 compounds of a supplemental metal, said filament containing, at ordinary temperatures, substantially only such gases as remain occluded therein at white incandescence.

7. A filament for electric vacuum lamps, containing osmium, and partly reduced oxid compounds of a rare metal earth, said filament containing, at ordinary temperatures, substantially only such gases as remain occluded therein at white incandescence.

8. A filament for electric vacuum lamps, containing osmium, partly reduced oxid compounds of a rare metal earth, and an oxid of a supplemental metal, said filament 120

125

130

containing, at ordinary temperatures, substantially only such gases as remain occluded therein at white incandescence.

9. A filament for electric vacuum lamps, containing osmium, and partly reduced oxid compounds of thorium, said filament containing, at ordinary temperatures, substantially only such gases as remain occluded therein at white incandescence.
10. A filament for electric vacuum lamps containing osmium, and partly reduced oxid compounds of a supplemental metal and an exterior coating of oxid, said exterior coating being of less conductivity than the partly reduced oxid.
11. A filament for electric vacuum lamps, containing osmium, partly reduced oxid

compounds of a supplemental metal, and an exterior coating of oxid, said exterior coating being of less conductivity than the partly reduced oxid.

12. A filament for electric vacuum lamps, containing osmium, partly reduced oxid compounds of a supplemental metal said partly reduced oxid being impregnated with an additional quantity of oxid and having a coating of said additional oxid.

In witness whereof I hereunto attach my signature, in the presence of two subscribing witnesses.

DR. CARL AUER VON WELSBACH.

Witnesses:

ADOLF GALLIA,  
L. HAILINGER.